

May 2, 1950

G. R. WAITKINS

2,506,049

LUBRICANT

Filed Dec. 18, 1946



INVENTOR

George R. Watkins

BY

*M. B. Lilly*  
Attorney

## UNITED STATES PATENT OFFICE

2,506,049

## LUBRICANT

George R. Waitkins, Flemington, N. J., assignor to  
 Battelle Memorial Institute, Columbus, Ohio, a  
 corporation of Ohio

Application December 18, 1946, Serial No. 717,032

13 Claims. (Cl. 252—46.7)

1

This invention relates to improved lubricants and, more particularly, to lubricants comprising a lubricating oil and a minor amount of a selenonophosphate.

When high-purity oils were introduced as lubricating oils, immersion oils, transformer oils, extreme pressure oils, and the like, they brought with them the problem of oil deterioration. These oils may deteriorate either by decomposition of the oil molecule, or by polymerization. A number of tests have been devised for measuring or indicating the exact degree to which any particular oil has deteriorated under given test conditions. For example, the presence of sludge is an indication of the formation of intermediate products through break-down of the oil molecule, whereas the acid number measures the extent to which the oil has been oxidized to produce free acids. An increase in viscosity indicates polymerization of the oil, and the carbon-content increase is a further measurement of the degree of decomposition of the oil. The formation of varnish upon surfaces which are oiled or subjected to the treatment of oil under high temperature or pressure indicates the tendency of the particular oil to form extremely hard polymers or resins upon metal surfaces which are being continuously exposed to the oil.

Oil is quite a complex mixture of compounds and one oil may frequently differ greatly from another, especially as to the particular manner in which it deteriorates or breaks down; that is, one oil may under test conditions produce a great deal of sludge with very little, if any, bearing loss, whereas another oil under identical test conditions will produce very little sludge but will show a high bearing loss. Consequently, it has been the practice in the art to produce additives having the general property of inhibiting oxidation or deterioration of the particular oil in question and which, as a special attribute, are designed to be especially effective in preventing sludge formation, increase in viscosity, high carbon residue, or some other particularly desirable property.

It is an object of this invention, therefore, to provide an improved lubricant consisting essentially of a lubricating oil and a minor amount of an oil additive for inhibiting the oxidation of oils.

Another object of this invention is to provide a lubricant containing as an addition to the lubricating oil a minor amount of an oil additive which markedly decreases the sludging of oils subject to metallic catalysts, heat, etc.

Still another object of the present invention is to provide a lubricant containing a minor

2

amount of an oil additive especially characterized by the property of reducing, and in some cases eliminating, lacquer formation on surfaces constantly exposed to the oil.

5 A further object of the present invention is to provide a lubricant containing as an addition to the lubricating oil a minor amount of an oil additive especially designed to so inhibit lubricating oils that engines employing the same will remain 10 clean and be relatively free from carbon, lacquer, and other foreign matter.

Other objects and advantages of the present invention will become apparent to those skilled in the art from the following detailed description 15 thereof when read in conjunction with the accompanying drawing in which the single figure is a graph illustrating the sludge-forming properties of a lubricant comprising the present invention.

20 In general, the present invention comprises a lubricant consisting essentially of a lubricating oil and a minor amount of an additive containing as an essential ingredient thereof an oil-insoluble organic selenonophosphate.

25 It has been found that oil-soluble organic selenonophosphates provide highly effective oil additives and are especially suitable as lubricating oil additives. These compounds have a general formula



where  $\text{R}_1$ ,  $\text{R}_2$ , and  $\text{R}_3$  are aryl, alkyl, alkaryl, or 35 aralkyl groups, and  $\text{X}$  may be hydrogen, a halogen, or the like. Usually, these groups are the same in any one compound as, for example, in tributyl selenonophosphate and triphenyl selenonophosphate, although they may all differ 40 from one another.

The selenonophosphates may be readily prepared by adding the theoretical amount of selenium to the corresponding phosphite. Since this reaction is highly exothermic, it is desirable to 45 place the phosphite container in an ice bath until the selenium has had an opportunity to dissolve. Following dissolution of the selenium, the ice bath may be removed and the solution stirred and filtered to remove any undissolved selenium. The 50 temperature of the solution will, of course, rise until the dissolution of the selenium is complete. In order to insure complete dissolution of all 55 selenium and reactance with the phosphite, the preferred procedure is to heat the solution from at least 5 to about 30 minutes at approximately 155° C. There are no particularly critical features in the preparation of the selenonophos-

phates, although heating for prolonged periods of time will produce a gummy, polymerized mass rather than the desired product. Among the compounds which have been successfully prepared in this manner are triamylselenonophosphate, triisoamylselenonophosphate, tri-3-ethyl

or high-carbon alkyl (tri-3-ethyl hexyl), di-substituted alkyl (di-n-butyl), low-carbon or short-chain alkyl (tri-butyl), a mixture of alkyl and aryl groups (diphenyl butyl), and aryl (tricresyl). Other types of selenonophosphate esters not above set forth may, of course, be employed.

TABLE 1  
*Indiana stirring oxidation tests on selenonophosphates*

| Additive                            | Average Values of Oil Deterioration Properties |      |      |                   |       |       |                            |       |         |    |    |    |
|-------------------------------------|------------------------------------------------|------|------|-------------------|-------|-------|----------------------------|-------|---------|----|----|----|
|                                     | Sludge                                         |      |      | Acid No. Increase |       |       | Percent Viscosity Increase |       |         | 24 | 48 | 72 |
|                                     | 24                                             | 48   | 72   | 24                | 48    | 72    | 24                         | 48    | 72      |    |    |    |
| Triamyl selenonophosphate           | 0.27                                           | 0.91 | 1.15 | 3.04              | 6.32  | 8.53  | 34.6                       | 90.6  | 136.4   |    |    |    |
| Triisoamyl selenonophosphate        | 0.11                                           | 0.11 | 0.20 | -0.39             | 0.21  | 1.40  | 7.10                       | 14.1  | 31.9    |    |    |    |
| Tri-3-ethyl hexyl selenonophosphate | 0.45                                           | 1.05 | 1.19 | 2.18              | 6.42  | 8.69  | 36.8                       | 109.7 | 153.5   |    |    |    |
| Di-n-butyl chloroselenonophosphate  | 0.10                                           | 0.31 | 1.02 | -0.62             | 2.00  | 10.30 | 8.91                       | 40.5  | 176.0   |    |    |    |
| Tributyl selenonophosphate          | 0.17                                           | 0.70 | 1.09 | 2.35              | 5.58  | 8.73  | 32.9                       | 88.5  | 149.9   |    |    |    |
| Diphenyl butyl selenonophosphate    | 0.11                                           | 0.25 | 0.92 | 0.42              | 2.38  | 10.07 | 6.57                       | 32.0  | 162.6   |    |    |    |
| Tricresyl selenonophosphate         | 0.20                                           | 0.58 | 1.01 | 1.69              | 4.94  | 9.32  | 19.1                       | 70.5  | 129.2   |    |    |    |
| None                                | 1.47                                           | 2.18 | (*)  | 12.82             | 18.53 | 23.02 | 196.8                      | 440.9 | 1,324.0 |    |    |    |

<sup>1</sup> Not sufficient sample remaining for test.

hexyl selenonophosphate, di-n-butyl chloroselenonophosphate, diphenyl butyl selenonophosphate, and tricresyl selenonophosphate. These compounds in amounts equal to 0.15 per cent selenium in the lubricant were added to a standard lubricating oil and tested in an Indiana stirring oxidation tester for periods of 24, 48, and 72 hours. The data are recorded in the following Table 1.

The data set forth in Table 1 under the heading "Sludge" represents the number of milliliters of sludge formed in each 10 milliliters of oil during the test period. It is at once apparent that all of the lubricants containing the selenonophosphate additives were much superior to the same lubricant without these additives. A comparison of the triamyl- and the triisoamylselenonophosphates indicates that branched chain ester groups may increase considerably the effectiveness of the additive.

The amount of additive added to the oil has been found not to be highly critical; however, there are certain preferred ranges which vary with the particular oil treated and the particular additive employed. Since these additives have different molecular weights and contain different percentages of the active ingredient, selenium, the per cent by weight of selenium in the final oil is used throughout the specification and accompanying claims as the basic standard. In the following Table 2, test results are shown which were obtained through the examination of an exemplary selenonophosphate, tributyl selenonophosphate, added to a usual type base oil, namely, Pennsylvania SAE 10. These tests were all run in accordance with the procedure known as Indiana stirring oxidation tests described in Industrial Engineering Chemistry, analytical edition, volume 13, page 317.

TABLE 2  
*Indiana stirring oxidation tests on tributyl selenonophosphate in Pennsylvania S.A.E. 10 oil*

| Test   | Per Cent Selenium | Initial | 24 Hours | 48 Hours | 72 Hours |
|--------|-------------------|---------|----------|----------|----------|
| Sludge |                   |         |          |          |          |
|        | 0.00              | 0       | 0        | 1.95     | 4.4      |
|        | 0.05              | 0       | 0        | 0.35     | 0.55     |
|        | 0.10              | 0       | 0        | 0.25     | 0.30     |
|        | 0.15              | 0       | 0        | 0.4      | 0.45     |
|        | 0.25              | 0       | 0        | 0.55     | 0.35     |
|        | 0.00              | 0.1     |          | 11.78    | 17.22    |
|        | 0.05              | 1.27    | 1.27     | 3.50     | 3.67     |
|        | 0.10              | 1.19    | 1.19     | 2.99     | 3.54     |
|        | 0.15              | 0.81    | 0.81     | 4.79     | 5.31     |
|        | 0.25              | 0.47    | 0.47     | 5.59     | 5.38     |
|        | 0.00              |         |          | 8.0      | 4.2      |
|        | 0.05              | 10      | 10       | 9.5      | 9.5      |
|        | 0.10              | 10      | 10       | 9.5      | 9.5      |
|        | 0.15              | 10      | 10       | 10       | 7        |
|        | 0.25              | 10      | 10       | 9        | 6        |
|        | 0.00              | 0       | 0        | 953      | 5        |
|        | 0.05              | 0       | 0        | 132      | 188      |
|        | 0.10              | 0       | 0        | 125      | 106      |
|        | 0.15              | 0       | 0        | 120      | 149      |
|        | 0.25              | 0       | 0        | 176      | 165      |

<sup>1</sup> Arbitrary assignment of numbers between 1 and 10 in which 10 designates a perfectly clean rod and 1 a very dirty rod.

The compounds shown in Table 1 represent widely variant types of organic selenonophosphate esters such as straight-chain alkyl (triamyl), branch-chain alkyl (triisoamyl), long-chain

The data above set forth in Table 2 in connection with sludge formation are graphically illustrated in the accompanying figure, wherein the 75 per cent of selenium in the oil (in the form of tri-

butyl selenonophosphate) is plotted against the milliliters of sludge formed per 10 milliliters of oil. It is at once evident that even minute quantities of selenium, as little as 0.01 per cent, effect a remarkable reduction in the amount of sludge formed. The greatest reduction of sludge formation, however, was achieved with this particular additive and particular oil in the range of from about 0.10 to about 0.15 per cent selenium. The upper limit of the amount of additive to be added is set primarily by the cost of the additive, although amounts greater than 0.25 per cent selenium had little, if any, added effect and in certain cases were somewhat less effective than smaller amounts. Although the data in Table 2 and the single figure refer to tributyl selenonophosphate, it has been found that the concentrations of selenium at which this additive may best be used is typical of the other oil-soluble organic selenonophosphate esters.

The effect of concentration variation of the selenium in the additive with respect to acid number, varnish formation, and viscosity increase, as shown in Table 2, indicates a marked improvement in the properties of the oil when the selenium is present in percentages varying from as little as 0.01 to 0.25 per cent. The smaller concentrations seem to be very effective in reducing the acid number, and further additions show very little improvement over the results achieved by adding 0.05 per cent selenium in the form of tributyl selenonophosphate. The decrease in varnish formation, on the other hand, reaches a maximum at about 0.15 per cent selenium. The lowest percentage increase in viscosity over a period of 48 hours was obtained with tributyl selenonophosphate additive containing 0.10 per cent selenium in the final oil.

Oil-soluble selenonophosphates comprising the present invention have been found to be especially desirable where cleanliness of the parts coming in contact with the oil was an essential feature and where minimum sludging of the oil was also requisite. Comparison of tributyl selenonophosphate with other commercial additives shown in the following Table 3 discloses that the selenonophosphate additive is greatly superior as respects its property to prevent lacquer formation and sludge formation. The data in the following Table 3 has been compiled using tributyl selenonophosphate at 0.1 per cent selenium concen-

TABLE 3  
Lauson engine tests  
[Demerits at 250 hours.]

|                                              | Tributyl Selenonophosphate | Commercial Additives |       |      |        |        |
|----------------------------------------------|----------------------------|----------------------|-------|------|--------|--------|
|                                              |                            | A                    | B     | C    | D      | E      |
| Skirt Lacquer (0-15)                         | 0.5                        | 2                    | 2     | 1    | 2      | 2      |
| Sludging (0-10)                              | 0                          | 2                    | 2     | 0    | 2      | 0      |
| Total Demerits                               | 0.5                        | 4                    | 4     | 1    | 4      | 2      |
| Observed and Measured Deposits:              |                            |                      |       |      |        |        |
| Skirt Lacquer Area                           | 5.0                        | 50                   | 30    | 20   | 30     | 30     |
| Skirt Lacquer Thickness                      | Ins.                       | 0.005                | 0.000 | 0    | 0.0002 | 0.0001 |
| Cylinder Head Deposits                       | Gms.                       | 0                    | 8.0   | 6.25 | 9.0    | 11.25  |
| Oil Consumption, Lbs./Hr.: Av. for 250 Hours |                            | .0028                | .0165 | .003 | .005   | .006   |
| Residue Tests:                               |                            |                      |       |      |        |        |
| Precipitation No. per cent                   | 0.75                       | 3.0                  | 4.0   | 3.0  | 2.0    | 5.0    |
| Original Conradson Carbon Residue do         | 0.39                       | 0.23                 | 0.46  | 0.51 | 0.56   | 0.38   |
| Conradson Carbon Residue, Final              | 3.88                       | 1.39                 | 4.8   | 4.96 | 2.0    | 3.88   |
| Naphtha Insolubles                           | do                         | 0.40                 | 0.93  | 2.6  | 2.36   | 0.72   |
| Carbon Disulphide Solubles                   | do                         | 0.16                 | 0.34  | 1.3  | 0.89   | 0.38   |
| Piston Rating: 1 (Cleanest) to 5             | 1                          | 1+                   | 2     | 2-   | 2      | 1+     |

tration in an SAE No. 20 lubricating oil. The oils were tested in Lauson single-cylinder engines using the high piston temperature procedure under the following operating conditions:

Speed ..... 1600 R. P. M.  
Load ..... 1.50 H. P. by two-blade fan  
Jacket temperature ..... 345 ± 5° F.  
Oil sump temperature ..... 225 ± 5° F.

- 5 Prior to the start of the test, a break-in run was made at 1200 R. P. M. for 30 minutes. Every 30 hours the engine was removed from its base and inspected and the crankpin bearings weighed.  
10 The engine was then re-assembled and the test continued to 240 hours, at the end of which time the used oil was analyzed for Conradson carbon residue and naphtha insolubles expressed in per cent by weight.  
15 The demerit system shown in the above Table 3 is purely an empirical method of establishing the extent to which the various parts of the motor exposed to the oil have been affected by lacquer, as well as the extent to which the oil has broken down to produce sludge. It is evident, however, from these tests that tributyl selenonophosphate is unquestionably superior to any of the other five commercial inhibitors or additives tested under similar conditions. Still more impressive  
20 are the tests showing the deposition of lacquer on the skirt and cylinder head. In these two areas, the test engines were substantially free from any deposit whatsoever, and the area covered by the skirt lacquer was only one-fourth as much as the area covered by the next cleanest additive. The precipitation number, an indication of sludge formation, was less than one-half of the next lowest additive. The formation of carbon in the oil to which tributyl selenonophosphate had been added appeared to be about average in comparison with all of the other additives tested, but a total of 0.56 gram of both naphtha insolubles and carbon disulphide insolubles were present in the sludge from the test  
30 oil to which tributyl selenonophosphate had been added as compared with the next lowest figure of 1.10 grams for additive B. It can be said from a perusal of Table 3 that the tributyl selenonophosphate additive, as representative of the organic selenonophosphates generally, is apparently superior to the other commercial additives as respects its property of maintaining surfaces exposed to the oil free from deposits.

40 Although the above tests refer particularly to lubricating oils, the use of the additives comprising the present invention is not limited to  
45

such oils but may be extended to electrical immersion oils, transformer oils, and the like. The following Table 4 discloses Indiana stirring oxidation tests run on electrical immersion oils. The

low acid number obtained by adding tributyl selenonophosphate to the electrical immersion oil tested is an indication of decrease in corrosive properties of the oil, whereas the low percentage of increase in viscosity obtained by adding this additive shows a decrease in the polymerization of the oil. Both of these factors are highly important, especially in large electrical installations where large quantities of oil are to be used over long periods of time.

The selenonophosphate additives may be used alone or in combination with other additives. For example, a mixture of tributyl selenonophosphate (0.10 per cent Se) and a 20 per cent solution of selenium dioxide (0.05 per cent Se) in benzyl alcohol proved to be particularly effective in reducing bearing corrosion.

It is apparent from the above detailed description thereof that the present invention comprises an improved lubricant consisting essentially of a lubricating oil and an oil-soluble organic selenonophosphate ester. By adding these esters, either alone or in combination with such additives as selenium dioxide, oils may be produced which are superior to those now in use in that they show less sludge formation and increased motor cleanliness.

TABLE 4  
*Indiana stirring oxidation tests over a period of 24 hours run on electrical immersion oils.*

| Additive                   | Per Cent Selenium | Sludge, ml. per 10 ml. of oil | Acid No. mg. KOH per g. oil | Viscosity Increase, Per Cent |
|----------------------------|-------------------|-------------------------------|-----------------------------|------------------------------|
| Tributyl selenonophosphate | 0.10              | 0                             | 7.28                        | 573                          |
| Do.                        | 0.15              | 0                             | 0.27                        | 128                          |
| None                       |                   | 8.0                           | 32.01                       | Solid                        |

What is claimed is:

1. An improved mineral oil composition comprising a major amount of a mineral oil and a minor amount sufficient to stabilize the oil against oxidation of an oil-soluble compound selected from the group consisting of alkyl, alkaryl, aralkyl, and aryl selenonophosphates.

2. A lubricant comprising a major amount of a mineral lubricating oil and a minor amount sufficient to stabilize the oil against oxidation of diphenyl butyl selenonophosphate.

3. A lubricant comprising a major amount of a mineral lubricating oil and a minor amount sufficient to stabilize the oil against oxidation of tributyl selenonophosphate.

4. A lubricant comprising a major amount of a mineral lubricating oil and from about 0.10 to about 0.15 per cent by weight of selenium as diphenyl butyl selenonophosphate.

5. A lubricant comprising a major amount of a mineral lubricating oil and from about 0.10 to about 0.15 per cent by weight of selenium as tributyl selenonophosphate.

6. A lubricant comprising a major amount of a mineral lubricating oil, about 0.10 per cent by weight of selenium as tributyl selenonophosphate and about 0.05 per cent by weight of selenium as selenium dioxide in benzyl alcohol.

7. A lubricant consisting essentially of a hydrocarbon lubricating oil and a minor amount sufficient to stabilize the oil against oxidation of an oil-soluble compound selected from the group consisting of alkyl, alkaryl, aralkyl and aryl selenonophosphates.

8. A lubricant consisting essentially of a hydrocarbon lubricating oil and a minor amount suffi-

cient to stabilize the oil against oxidation of a mixture of an oil-soluble compound selected from the group consisting of alkyl, alkaryl, aralkyl and aryl selenonophosphates, and selenium dioxide.

9. A lubricant consisting essentially of a hydrocarbon lubricating oil and an oil-soluble compound selected from the group consisting of alkyl, alkaryl, aralkyl, and aryl selenonophosphates in a concentration such that the resulting lubricant contains from at least 0.01% to about 0.25% by weight of selenium.

10. A lubricant consisting essentially of a hydrocarbon lubricating oil and an oil-soluble compound selected from the group consisting of alkyl, alkaryl, aralkyl and aryl selenonophosphates, in a concentration such that the resulting lubricant contains from 0.10% to 0.15% by weight of selenium.

11. A lubricant consisting essentially of a hydrocarbon lubricating oil and a mixture of an oil-soluble compound selected from the group consisting of alkyl, alkaryl, aralkyl, and aryl selenonophosphates in a concentration such that the resulting lubricant contains about 0.10% by weight of selenium as said selenonophosphate, and about 0.05% by weight of selenium as selenium dioxide dissolved in an organic alcohol.

12. A lubricant consisting essentially of a hydrocarbon lubricating oil and a minor amount sufficient to stabilize the oil against oxidation of an oil-soluble organic compound of the type



in which  $R_1$  and  $R_2$  represent alkyl, aryl, alkaryl, or aralkyl groups and  $X$  represents hydrogen or a halogen atom.

13. An improved mineral oil composition comprising a major amount of a mineral oil and a minor amount sufficient to stabilize the oil against oxidation of an oil soluble organic selenonophosphate compound of the type



in which  $R_1$  and  $R_2$  represent alkyl, aryl, alkaryl or aralkyl groups and  $X$  represents a halogen atom.

GEORGE R. WAITKINS.

#### REFERENCES CITED

The following references are of record in the file of this patent:

#### UNITED STATES PATENTS

| Number    | Name         | Date           |
|-----------|--------------|----------------|
| 2,157,452 | Humphreys    | May 9, 1939    |
| 2,355,106 | Prutton      | Aug. 8, 1944   |
| 2,359,270 | Shutt et al. | Sept. 26, 1944 |
| 2,359,331 | Reiff        | Oct. 3, 1944   |